

A. J. HARRY.

METHOD AND APPARATUS FOR TREATING SAWS WITH HEAT,  
APPLICATION FILED FEB. 17, 1921.

1,429,138.

Patented Sept. 12, 1922.  
2 SHEETS—SHEET 1.



Fig. 1,



Fig. 2,

WITNESSES

*Edw. Thorpe.*  
*Robert J. Hulsizer*

INVENTOR

*Albert J. Harry*  
BY  
*Munn Co.*  
ATTORNEYS

A. J. HARRY.

METHOD AND APPARATUS FOR TREATING SAWS WITH HEAT.

APPLICATION FILED FEB. 17, 1921.

1,429,138.

Patented Sept. 12, 1922.

2 SHEETS—SHEET 2.

*Fig. 3,*



*Fig. 4.*



Albert J. Harry  
BY  
Munro  
ATTORNEYS

## UNITED STATES PATENT OFFICE.

ALBERT JOSEPH HARRY, OF EAST CLEVELAND, OHIO.

## METHOD AND APPARATUS FOR TREATING SAWS WITH HEAT.

Application filed February 17, 1921. Serial No. 445,659.

*To all whom it may concern:*

Be it known that I, ALBERT J. HARRY, a citizen of the United States, and a resident of East Cleveland, in the county of Cuyahoga and State of Ohio, have invented a new and Improved Method and Apparatus for Treating Saws with Heat, of which the following is a full, clear, and exact description.

10. This invention relates to apparatus for treating saws with heat, and has for an object the provision of a simple and economically manufactured, compact and efficient apparatus for treating saws, particularly disk saws, to a definite temperature immediately after they have been taken from the furnace.

Another object is to provide an efficient and simple apparatus in which the saws 20. while being so treated to a definite temperature can be kept straight and flat and are, therefore, not liable to warp or bend as is sometimes the case.

A further object resides in the provision 25. of a process or series of steps whereby the high-speed steel of which the saws are made is produced in a better condition by the particular process adopted than heretofore has been the case.

30. A still further object resides in the particular construction and arrangement of parts and in the particular sequence of steps in the process applied, hereinafter claimed, and shown in the accompanying drawings.

35. In general, it is known to be old to quench high-speed steel, of which saws are made, in a bath at 1150° F., thus tempering it at the same time to the maximum toughness. Hitherto it has been customary to put heavy articles, where possible, into a lead bath at 1150° F. directly from the furnace at 2250° F.

In accordance with my method, however, 45. I adopt a somewhat similar process with the additional feature that during the time that the saws, or other high-speed steel articles, are being subjected to the lower temperature after coming from the furnace, they are subjected to a certain pressure between flat surfaces to keep them straight. These flat sur-

faces are also heating elements which subject the article to the desired temperature for the proper length of time.

The heating surfaces between which the flat articles of steel are subjected to pressure 55 form parts of a press and are constructed as electrical heating elements in a manner to be hereinafter described.

The invention is illustrated in the drawings, of which—<sup>60</sup>

Figure 1 represents a front view of the apparatus by which the process embodying my invention is applied;

Figure 2 is a side view of the apparatus;

Figure 3 is a plan view, with a portion cut 65 away, of one of the heating plates; and

Figure 4 is a section taken on the line 4—4 of Figure 3.

The preferred embodiment of my invention, as shown in the drawing, comprises a 70. press having a base plate 1 which can be attached in any suitable manner to a floor from which extends a vertical supporting column or rib 2 to the upper end of which a top plate 3 is connected. Between the plates 75 1 and 3 a pair of spaced, vertically extending, parallel guide bars 4 are disposed. These guide bars are adapted to receive apertured lugs, such as 5, disposed on opposite sides of a slidable heating unit 6. This heating unit is kept in its vertical movement by the bars 4 and has on its upper surface a journal block 7 to which is pivoted a connecting rod 8. This rod 8 is pivotally connected to a crank arm 9 which is pivoted at 10 in the upper block or top plate 3 and forms part of a handle member 11. The operation of the handle member in one direction or the other moves the upper sliding heating plate 6 toward and away from a similar heating unit such as 12 which may be securely fastened in any suitable manner to the base block or plate 1.

In the process which is applied by means of the use of apparatus of this general type, 95 high-speed steel articles, preferably flat articles such as disk saws, are initially treated in a furnace to a temperature of approximately 2250° F., after which they are quenched by being subjected to a lower tem- 100

perature of substantially  $1150^{\circ}$  F. Ordinarily this second step in the treatment is effected by plunging the saws into an oil bath at room temperature, after which the saws are drawn again in a lead bath at  $1150^{\circ}$  F. However, in this particular form of the second step, no means are provided for keeping the saws under pressure whereby they may be kept straight and prevented from warping. However, in accordance with my invention, I place the saws, or other articles, as soon as they are taken from the furnace, between the heating plates such as 6 and 12 and subject them to a definite pressure for a proper length of time, and during this time supply heat to the plates 6 and 12 by electrical means so that the saws or other articles are slowly cooled from  $2250^{\circ}$  F. down to  $1150^{\circ}$  F., which is approximately the temperature of the heating plates 6 and 12. I find that by thus treating the saws they are maintained straight and do not warp and that their mechanical and structural condition is such that they require no further heat treatment and are free from strains. Saws treated in this particular manner are found to be extremely tough and hard and are capable of doing much more work in use. The saving of time and labor by adopting this particular process is also considerable.

In Figures 3 and 4, I show one of the heating units or plates, such as 6 or 12, and a description of this will suffice for both since they are substantially identical. The plate shown in Figures 3 and 4 is in the form of a shell having a flat surface 13, preferably made of nichrome or Monel metal, which does not deteriorate under high temperatures, which is bent over along its circumference and provided with a flange such as 14. This flange portion is provided at intervals with ear portions, such as 15, suitably pierced with apertures and connected up to a base or cover plate 16 made of any suitable material, such as steel, provided with similar ears 17. The cover 16 and plate 13 are held together by bolts 18 co-operating with the ears 15 and 17. As above described, the shell is in the form of a shallow circular cup. Within this shell, and made integral with the plate 13, are a plurality of radially extending reinforcing ribs such as 19 which help to strengthen the plate. These ribs are formed integrally with the shell, which may be cast. These reinforcing ribs 19 extend from the inner face of the heating surface 13 to the bottom plate 16. The resistor element, which is in the form of a suitably coiled and spaced wire 20, is disposed beneath but spaced from the heating plate 13 and is in the form of a wire made preferably of some material such as nichrome. This wire is disposed in suitably provided grooves such as 21 in the upper surface of a layer of refractory mate-

rial, such as fire clay, and which is represented by the numeral 22. Beneath this layer of fire clay is a layer of soft asbestos or magnesia 23, and beneath this layer is a piece of hard asbestos lumber such as 24. 70 This piece 24 lies against the bottom plate of the cover 16. A suitable connection, such as 25, extends from the resistor element 20 to an outside power source which offers the required amount of electric current to heat 75 the plate 13 to the desired temperature, which in this case is approximately  $1125^{\circ}$  F. The surface heat to  $1125^{\circ}$  F. instead of  $1150^{\circ}$  is to allow for a higher heating of the saw.

In order to accurately determine the temperature of the heating plate, I may provide any suitable form of pyrometer, which can be inserted or attached to each heating plate in any desired manner, to indicate the temperature thereof. This particular construction is not shown for the reason that it may be provided in any particular manner and form no essential part of my invention.

The process in which this apparatus is used is simply to take the saw or other article from the furnace at  $2250^{\circ}$  F. and place it in this press and hold it therein under a suitable pressure the proper length of time until the temperature of the heating plates is reached by the saw or article. 95 After this temperature is reached, the saw can be removed from the press and can be then cooled in air or may be disposed of in any other way following this operation. No further treatment is required of the 100 articles, and they are capable of operating under the conditions above mentioned and possess the above-mentioned highly advantageous qualities due to the treatment they have received.

It is, of course, apparent that minor modifications in the materials and arrangement of the structure above mentioned can be adopted without departing from the spirit of the invention as set forth.

What I claim is:

1. A method of treating flat metallic articles such as saws, which comprises subjecting them to a high heat, then substantially immediately subjecting them to a 115 lower heat, and subjecting them to pressure during their subjection to the lower heat.

2. A method of treating flat metallic articles such as steel saws, which comprises subjecting them to a high heat, then substantially immediately subjecting them to a lower heat, subjecting them to pressure during their subjection to the lower heat, and then permitting them to cool in the atmosphere free from pressure and heat.

3. A method of treating flat metallic articles such as high-speed steel saws, which comprises subjecting them to a temperature of substantially  $2250^{\circ}$  F., then substantially immediately subjecting them to a tempera-

ture of 1150° F., and subjecting them to a substantially immediately subjecting them to a small pressure during their subjection to a temperature of 1150°, subjecting them to a this lower temperature.

4. A method of treating flat metallic articles such as high-speed steel saws, which comprises subjecting them to a temperature of substantially 2250° F., then sub-stantially immediately subjecting them to a small pressure during their subjection to a this lower temperature, and then allowing them to cool in an atmosphere free of both pressure and heat.

ALBERT JOSEPH HARRY.